

# UNITED STATES PATENT OFFICE.

JAMES R. ROSE, OF EDGEWORTH, PENNSYLVANIA, AND JOHN HARRIS, OF LAKEWOOD,  
OHIO, ASSIGNORS TO CARBO-OXYGEN COMPANY, OF PITTSBURGH, PENNSYLVANIA,  
A CORPORATION OF DELAWARE.

## GASEOUS FUEL.

1,404,225.

Specification of Letters Patent. Patented Jan. 24, 1922.

No Drawing.

Application filed December 26, 1919. Serial No. 347,452.

To all whom it may concern:

Be it known that we, (1) JAMES R. ROSE,  
(2) JOHN HARRIS, citizens of the United  
States, residing at (1) Edgeworth, (2)  
5 Lakewood, in the county of (1) Allegheny,  
(2) Cuyahoga, and State of (1) Penn-  
sylvania, (2) Ohio, have invented a certain  
new and useful Improvement in Gaseous  
Fuel, of which the following is a full, clear,  
10 and exact description.

This invention relates to gaseous fuel, and  
more particularly to a fuel which is espe-  
cially adapted for the purpose of cutting  
metals with great rapidity, where extreme  
15 cleanliness of cutting is not essential. A use  
for which our gas is particularly well suited  
is for the cutting of scrap iron.

We obtain a gas having the above desire-  
able characteristics by mixing with hydro-  
20 gen, as a combustible base, propane and  
carbon monoxide in the proportions of from  
2 $\frac{1}{2}$ % to 12 $\frac{1}{2}$ % by volume each of such pro-  
pane and carbon monoxide to the hydrogen  
constituent. The carbon monoxide serves to  
25 increase slightly the temperature produced  
by the combustion of hydrogen alone.  
Furthermore, the gaseous mixture produces  
within the burning hydrogen a visible cone  
which enables the operator to adjust the pro-  
30 portions of the gases and the combustion-  
supporting oxygen as may be necessary and  
to apply the flame in the most advantageous  
manner to the work. Both the volume of  
the flame and the heat units produced by  
35 the combustion of the mixture are greater  
than are produced by the combustion of  
hydrogen alone, but are lower than usually  
required for operating on heavy masses of  
metal and for cutting cast iron and steel  
40 and corroded, dirty and slaggy iron and  
steel. However, our gaseous mixture is

capable of cutting with much greater  
rapidity than can be accomplished by gases  
having such higher carbon content.

According to Richards on Metallurgical 45  
Calculations, published in 1908, the flame  
temperature produced by the combustion of  
the aforesaid gases will be above 3200° C.,  
and the variations in the percentages of the  
said gases will cause approximately the 50  
following variations in the net B. T. U. per  
cubic foot of mixture and in the cubic feet  
of oxygen required for the combustion of a  
cubic foot of such mixture:

No. 1 mixture, 95% H. with 2 $\frac{1}{2}$ % each of 55  
propane and carbon monoxide; net B. T.  
U. is 348; cu. ft. of oxygen .613.

No. 2 mixture, 75% H. with 12 $\frac{1}{2}$ % each 60  
of propane and carbon monoxide; net B. T.  
U. is 567; cu. ft. of oxygen 1.125.

Having thus described our invention,  
what we claim is:

1. A gas for cutting, welding and heating  
purposes consisting of a mixture of carbon  
monoxide and propane with hydrogen in 65  
the proportions of from 2 $\frac{1}{2}$ % to 12 $\frac{1}{2}$ % by  
volume each of carbon monoxide and pro-  
pane to hydrogen.

2. A gas for cutting, welding and heating  
purposes consisting of a mixture of propane 70  
and carbon monoxide with hydrogen in pro-  
portions not substantially less than 5% by  
volume of such combined gases to the hydro-  
gen and not materially more than 25% of  
such combined gases to the hydrogen, the 75  
propane and carbon monoxide being present  
in the proportions of at least 2 $\frac{1}{2}$ % each in  
such mixture.

In testimony whereof, we hereunto affix  
our signatures.

JAMES R. ROSE.  
JOHN HARRIS.